

Jan. 12, 1937.

A. BRANDT

2,067,824

TORPEDO

Filed March 16, 1935

Fig. 1



Fig. 2



Fig. 3



August Brandt  
by

Dean, Fairbank, Huoch & Foster  
Attorneys.

## UNITED STATES PATENT OFFICE

2,067,824

## TORPEDO

August Brandt, Ballenstedt/Harz, Germany

Application March 16, 1935, Serial No. 11,521  
In Germany September 13, 1933

4 Claims. (Cl. 102—25)

The invention relates to torpedoes of any shape which produce explosive effects and coruscating lighting effects if the body is ignited. It is a molded body for instance in the form of a bar, a rod, a plate, a pyramid, or any other geometrical form. The mass of the torpedo is non-poisonous.

The new torpedo body consists of a binding material and flux admixed with a pyrotechnical mixture including a carbon bearer, an oxygen bearer and a light metal alloy. The pyrotechnical mixture may consist of shellac, saltpetre, potassium chlorate or perchlorate and aluminum, magnesium, alloy. The binding material may be dextrine.

The flux materials are according to the invention such substances as effect a sintered ash, preferably fluorine compounds, fluorine salts or mixtures thereof. Alkali fluorides, fluorides of light metals as aluminum and zinc, fluorides of heavy metals as iron, copper and the like, also fluorides of alkaline earth metals are useful for the purpose. Compound fluorides such as silicic fluorides, boric fluorides and the like are also of utility and may be applied alone or admixed with the simple fluorides.

Advantageously double salts of hydrofluoric acid may be used as flux or sintering or scorifying addition. Alkali or aluminum or combinations thereof may serve as the metallic element of the fluoride.

A preferred flux or flux ingredient is the material known as cryolite.

An illustrative moldable mixture serviceable for the purpose is:

|                                             | Parts |
|---------------------------------------------|-------|
| Cryolite                                    | 40    |
| Shellac                                     | 40    |
| Saltspetre                                  | 15    |
| Dextrine                                    | 12    |
| Potassium chlorate or potassium perchlorate | 180   |
| Aluminum-magnesium-alloy                    | 170   |

The aluminum magnesium alloy consists preferably of 50 parts of magnesium and 50 parts of aluminum.

The torpedoes may be provided with a pyrophoric mass ignited by friction. 5

In the accompanying drawing is shown illustrative examples of the new torpedoes.

Fig. 1 is a perspective view of a rod shaped torpedo. 10

Fig. 2 is a plan view of a plate shaped torpedo, and

Fig. 3 is a perspective view of a pyramidal torpedo. 15

In each of the figures of the drawing 1 is the body which is molded from a pyrotechnical mixture containing a binder and a flux as described above, and 2 are pyrophoric heads ignitable by friction. 20

What I claim is:

1. A molded pyrotechnic device of non-poisonous character including a pyrotechnical mixture of an alloy of metallic aluminum and magnesium, a carbon bearing material and an oxygen releasing material together with a flux and a binder. 25

2. The combination recited in claim 1 in which the flux is an alkaline fluoride.

3. A molded torpedo consisting of approximately 40 parts of cryolite, 40 parts of shellac, 15 parts of saltpetre, 12 parts of dextrine, 180 parts of potassium chlorate and 170 additional parts of aluminum-magnesium-alloy. 30

4. The torpedo claimed in claim 3 in which the alloy ingredient is of substantially equal parts of aluminum and magnesium. 35

AUGUST BRANDT. 40